

July 18, 1950

E. J. ABBOTT

2,515,172

SPLICING THREADS

Filed April 30, 1948



Inventor  
Edward J. Abbott  
by Roberts, Cushman & Grood  
Atty's.

## UNITED STATES PATENT OFFICE

2,515,172

## SPLICING THREADS

Edward James Abbott, Wilton, N. H., assignor to  
 Abbott Machine Company, Wilton, N. H., a corporation of New Hampshire

Application April 30, 1948, Serial No. 24,114

19 Claims. (Cl. 57—159)

1

This invention relates to the splicing of thread, particularly single-ply thread either intended to be used as single-ply thread or subsequently twisted together with another ply or plies.

In the handling of thread it is often necessary to join two lengths together, such for example as to join the leading end of one bobbin of thread to the tail end of another bobbin of thread, or to join together two pieces from between which some imperfection, such as a slub, has been cut out.

The usual commercial practice is to tie two such threads together by knotting. However, in many cases, knots are objectionable. Difficulties with yarn tangling in being unwound from bobbins are sometimes attributable to the presence of knots in the thread. Moreover, knots have a tendency to catch in various elements of thread handling machinery, such as the heddles and reeds of looms, and in the needles of knitting machines. Moreover, when they appear in the finished fabric, knots often either have to be buried out of the fabric, or else constitute a visible imperfection in the fabric.

The invention accordingly aims to provide for joining together two pieces of thread with a joint of improved strength and which avoids the objectionable features of knots and of previously used splices.

Other objects of the invention and features of advantage will be apparent from this specification and its drawings wherein the invention is explained by way of example.

In the drawings, in which all the figures are enlarged, but not accurately to scale,

Fig. 1 is a diagrammatic view showing two pieces of single-ply thread which are to be joined by use of this invention;

Fig. 2 is a diagrammatic view showing the two pieces of thread after twist has been displaced from an end portion of each into the remaining part of the piece of thread;

Fig. 3 is a diagrammatic view showing the two end portions disposed in overlapping relation in contact with each other;

Fig. 4 is a diagrammatic view showing the end portions of Fig. 3 after drafting; and

Fig. 5 is a diagrammatic view showing the completed joint after the twist has been returned into the drafted material.

An advantage of the present invention lies in its ability to cause the splice to have as long a length as may be desirable, having in mind the type and quality of fibers, the twist, and the size of the thread to be joined. The invention thus

2

overcomes certain practical limitations which in the past have seriously limited the strength of joints.

I have discovered that the mere fact that a joint of a spliced thread resembles in appearance the original parts of the thread does not at all insure that the joint will have adequate strength. For instance, if two cut pieces of thread are untwisted near their ends, removal of the short-length fibers which result from the cutting produces a tapered or frayed portion, and if the two such tapered portions are overlaid and twisted together, a joint resembling the original thread will result. However, unless adhesive is added a joint so produced has very little strength; and it may reasonably be concluded that in such a joint the cohesion of individual fibers is deficient as compared to the cohesion of fibers within the original unspliced pieces of thread.

20 The present invention involves a drafting of untwisted end portions of the thread and a twisting together of these drafted portions.

The invention may be practiced by machinery or by hand manipulation of the thread, and in 25 hand manipulation simple clamps or weights may advantageously be used to hold the material in an untwisted state preparatory to and during the drafting.

In practicing the present invention the twist is first substantially removed from an end portion 30 of each of the two pieces of threads to be joined. Preferably, twist is removed from an end portion of each thread exceeding in length the average fiber length of the fibers of which the thread consists, or still better, from an end portion

35 of each thread exceeding even the maximum fiber length. Thus, with cotton having an average fiber length of 1 inch the twist may for instance be removed from a 2 inch length of each thread end. Thus the untwisted portion consists

40 in large part of an average assortment of the fibers of the original thread, untwisted, and with a large part and often the preponderant part of the fibers of the untwisted portion not extending into the remaining twisted main portion of the thread, but floating, so to speak, in the untwisted end portion and capable of lengthwise shift by a drafting operation.

In the preferred procedure, the untwisted portions of the two threads, which are to form the

50 joint, thus consist largely of fibers which have neither been cut or broken, so that the joint does not need to depend for strength upon such shortened and less desirable fibers.

55 Removal of the twist from an end portion of

each of the two threads is preferably, and most expeditiously, accomplished by displacing this twist into the remaining part of such thread and holding it there while the end portions are required to be in an untwisted state. Thus, with the end of thread 11 held at the line 13-13, the twist originally in the portion of thread 11 between lines 13-13 and 14-14 is forced to the left (as shown in Fig. 2) into the main body portion of thread 11, where the twist therefore becomes somewhat steeper than originally, and the thread 11 is then held at the line 14-14, temporarily preventing the twist from returning into the portion L between lines 13-13 and 14-14.

A similar untwisting operation is performed either simultaneously or successively upon the corresponding end portion of thread 12, with the result that the corresponding end portions of both threads are in an untwisted state, and when this untwisting is accomplished by displacement of twist into the main portions of the threads, the twist that was originally in the end portions augments the twist originally present in the remaining main portions of thread.

It will be understood that during the operation of removing the twist from the end portions of the threads, the threads need not necessarily yet be oppositely directed nor parallel as shown in Fig. 2, but they are so shown in Fig. 2 because it is more convenient to hold and handle them in this manner.

After removal of the twist from the end portions of the two threads, the two such end portions are drafted and are twisted together. The strength of the joint is considerably improved if this drafting of the two untwisted end portions is performed simultaneously upon the two end portions while these end portions are in contact with each other, and this preferred procedure will be described.

Accordingly the two, oppositely disposed untwisted end portions are shown as overlapped in contact with each other in Fig. 3 preparatory to the drafting. Thereupon the two end portions, held in an untwisted state, are drafted together, producing an elongated condition of each of these untwisted portions as diagrammatically shown in Fig. 4 and a corresponding material reduction in thickness of the splice eventually resulting, as compared to merely combining such end portions without drafting.

Drafting largely reduces the extent to which fibers or ends of fibers are wrapped around the bundle of fibers of each end portion, and the drafting brings the fibers into a straight condition in which they are best adapted to become cohered with their neighboring fibers. When, as in the preferred example, the drafting is performed simultaneously on the two ends which are overlapped and in contact, the line of demarcation between the two ends, diagrammatically shown in Fig. 3, substantially disappears as a result of the drafting, as indicated in Fig. 4. Cohesion of fibers stemming from the opposite threads is thus promoted and the strength of the ultimate joint is increased accordingly.

The cohesion of fibers stemming from the opposite threads can be further promoted by increasing the total length of the untwisted portions that are superposed for the drafting, and the ability of the process to make the joint as long as may be desired is advantageous in making it possible for the two overlapped portions of the joint to lose their initial character of sepa-

rate plies and contribute to the strength of the joint by cohesion of individual fibers.

Upon completion of the drafting, twist of the same or approximately the same degree as the twist of the original thread is imparted to the drafted material, producing the joint shown in Fig. 5 in which all parts of the united thread have substantially the same degree of twist. When the removal of twist from the end portions of the thread has been accomplished by displacing the twist into the remaining main portions of thread and holding it there during the drafting, the twist can readily be restored to the drafted material by merely removing the restraint which has been applied at lines 13-13 and 14-14 and so allowing the twist to run back into the drafted material from both main portions of the thread.

The drafting operation, described above, should be carried on to an extent such that after the restoration of twist the retwisted material of the joint has approximately the diameter of the main portions of the joined threads, and this result is secured when the draft applied to the untwisted portions is a draft of approximately two times, the length L of Fig. 2 being drafted to a length of 2 times L in Fig. 4.

When, as indicated above, each untwisted end which is drafted in the process is long enough so that a large part of its fibers comprise an average assortment of fibers (with reference to the fibers of the original thread) and so that a large part of its fibers do not extend into the still-twisted main portion of thread but float in the untwisted portion, the composite thread of the drafted joint can closely conform to the original thread in fiber distribution.

The joint produced by this invention requires no adhesive, having adequate strength as made without adhesive. The joint moreover, is practically indistinguishable in size and appearance from the original threads, excepting that the two slight tail portions may, without detriment, protrude from the joined thread, as shown in Fig. 5.

I claim:

1. Method of splicing two threads of twisted fibers comprising removing twist from an end portion of each of the threads, drafting each untwisted end portion, and twisting the drafted end portions together, the drafting of the end portions being carried to an extent sufficient to represent a material reduction in thickness of the resulting splice, as compared to combining such end portions without drafting.

2. Method of splicing two threads of twisted fibers comprising removing twist from an end portion of each of the threads for a sufficient length so that fibers of average length with reference to the fibers of the original thread are contained substantially free from twist within such untwisted portion, drafting each untwisted end portion and twisting the drafted end portions together, the drafting of the end portions being carried to an extent sufficient to represent a material reduction in thickness of the resulting splice, as compared to combining such end portions without drafting.

3. Method of splicing two threads of twisted fibers comprising removing twist from an end portion of each of the two threads, disposing the two untwisted end portions in overlapped relation, oppositely directed, and while so disposed drafting said untwisted overlapped portions, and thereafter restoring twist into the drafted material, the drafting of the end portions being carried to an extent sufficient to represent a mate-

rial reduction in thickness of the resulting splice, as compared to combining such end portions without drafting.

4. Method of splicing two threads of twisted fibers comprising removing twist from an end portion of each of the two threads, disposing the two untwisted end portions in overlapped relation, oppositely directed, and while so disposed intermingling the fibers of the two overlapped end portions by subjecting said fibers to a drafting operation, and thereafter restoring twist into the drafted material, the drafting of the end portions being carried to an extent sufficient to represent a material reduction in thickness of the resulting splice, as compared to combining such end portions without drafting.

5. Method of splicing two threads of twisted fibers comprising removing twist from an end portion of each of the two threads, overlapping with each other a sufficient length of each untwisted end portion so that untwisted fibers of average length with reference to the fibers of the original thread are overlapped with similar untwisted fibers of the other end portion, and while so disposed drafting said untwisted overlapped portions, and thereafter restoring twist into the drafted material, the drafting of the end portions being carried to an extent sufficient to represent a material reduction in thickness of the resulting splice, as compared to combining such end portions without drafting.

6. Method of splicing two threads of twisted fibers comprising removing twist from an end portion of each of the two threads, said end portion in which the twist is removed being greater in length than the average length of the constituent fibers of its thread, disposing the two untwisted end portions in overlapped relation, oppositely directed, and while so disposed drafting said untwisted overlapped portions, and thereafter restoring twist into the drafted material, the drafting of the end portions being carried to an extent sufficient to represent a material reduction in thickness of the resulting splice, as compared to combining such end portions without drafting.

7. Method of splicing two threads of twisted fibers comprising removing twist from an end portion of each of the two threads, said end portion in which the twist is removed being at least as long as the maximum length of the constituent fibers of its thread, disposing the two untwisted end portions in overlapped relation, oppositely directed, and while so disposed drafting said untwisted overlapped portions, and thereafter restoring twist into the drafted material, the drafting of the end portions being carried to an extent sufficient to represent a material reduction in thickness of the resulting splice, as compared to combining such end portions without drafting.

8. Method of splicing two threads of twisted fibers comprising removing twist from an end portion of each of the two threads, said end portion in which the twist is removed being sufficiently long that a large part of the fibers therein do not extend into the remaining twisted portion of the thread, disposing the two untwisted end portions in overlapped relation, oppositely directed, and while so disposed drafting said untwisted overlapped portions, thereafter restoring twist into the drafted material, the drafting of the end portions being carried to an extent sufficient to represent a material reduction in thickness of the resulting splice, as com-

pared to combining such end portions without drafting.

9. Method of splicing two threads of twisted fibers comprising displacing twist from an end portion of each of the two threads into the remaining part of such thread, disposing the two untwisted end portions in overlapped relation, oppositely directed, and while so disposed drafting said untwisted overlapped portions, and thereafter restoring twist into the drafted material, the drafting of the end portions being carried to an extent sufficient to represent a material reduction in thickness of the resulting splice, as compared to combining such end portions without drafting.

10. Method of splicing two threads of twisted fibers comprising displacing twist from an end portion of each of the two threads into the remaining part of such thread, disposing the two untwisted end portions in overlapped relation, oppositely directed, and while so disposed drafting said untwisted overlapped portions, and thereafter allowing twist to run from said remaining parts of said threads into the drafted material, the drafting of the end portions being carried to an extent sufficient to represent a material reduction in thickness of the resulting splice, as compared to combining such end portions without drafting.

11. Method of splicing two threads of twisted fibers comprising displacing twist from an end portion of each of the two threads into the remaining part of such thread, disposing the two untwisted end portions in overlapped relation, oppositely directed, and while so disposed drafting said untwisted overlapped portions, and thereafter restoring twist into the drafted material, the drafting being carried to an extent such that after restoration of twist the retwisted material has approximately the diameter of the main portions of the joined threads.

12. Method of splicing two threads of twisted fibers comprising displacing twist from an end portion of each of the two threads into the remaining part of such thread, disposing the two untwisted end portions in overlapped relation, oppositely directed, and while so disposed drafting said untwisted overlapped portions with a draft of approximately two times, and thereafter restoring twist into the drafted material.

13. Method of splicing two threads of twisted fibers comprising removing twist from an end portion of each of the threads, drafting each untwisted end portion, and twisting the drafted end portions together, the drafting of the end portions being carried at least to an extent of approximately two.

14. Method of splicing two threads of twisted fibers comprising removing twist from an end portion of each of the threads for a sufficient length so that fibers of average length with reference to the fibers of the original thread are contained substantially free from twist within such untwisted portion, drafting each untwisted end portion and twisting the drafted end portions together, the drafting of the end portions being carried at least to an extent of approximately two.

15. Method of splicing two threads of twisted fibers comprising removing twist from an end portion of each of the two threads, disposing the two untwisted end portions in overlapped relation, oppositely directed, and while so disposed drafting said untwisted overlapped portions, and thereafter restoring twist into the drafted ma-

aterial, the drafting of the end portions being carried at least to an extent of approximately two.

16. Method of splicing two threads of twisted fibers comprising removing twist from an end portion of each of the two threads, said end portion in which the twist is removed being greater in length than the average length of the constituent fibers of its thread, disposing the two untwisted end portions in overlapped relation, oppositely directed, and while so disposed drafting said untwisted overlapped portions, and thereafter restoring twist into the drafted material, the drafting of the end portions being carried at least to an extent of approximately two.

17. Method of splicing two threads of twisted fibers comprising removing twist from an end portion of each of the two threads, said end portion in which the twist is removed being at least as long as the maximum length of the constituent fibers of its thread, disposing the two untwisted end portions in overlapped relation, oppositely directed, and while so disposed drafting said untwisted overlapped portions, and thereafter restoring twist into the drafted material, the drafting of the end portions being carried at least to an extent of approximately two.

18. Method of splicing two threads of twisted fibers comprising removing twist from an end portion of each of the two threads, said end portion in which the twist is removed being sufficiently long that a large part of the fibers therein do not extend into the remaining twisted portion of the thread, disposing the two untwisted end portions in overlapped relation, oppositely directed, and while so disposed drafting said untwisted overlapped portions, thereafter restoring twist into the drafted material, the drafting of the end portions being carried at least to an extent of approximately two.

19. Method of splicing two threads of twisted fibers comprising displacing twist from an end portion of each of the two threads into the remaining part of such thread, disposing the two untwisted end portions in overlapped relation, oppositely directed, and while so disposed drafting said untwisted overlapped portions, and thereafter restoring twist into the drafted material, the drafting of the end portions being carried at least to an extent of approximately two.

EDWARD JAMES ABBOTT.

No references cited.